

(No Model.)

J. J. WILLIAMSON.

METHOD OF MAKING ELECTRICAL CONDUCTORS.

No. 319,536.

Patented June 9, 1885.

Fig. 1.  
α



Fig. 2.



Fig. 3.



Witnesses:

J. M. Dolan  
Geo. R. Tolman

Inventor:  
J. J. Williamson  
by his attys  
Clarke & Baynard.

# UNITED STATES PATENT OFFICE.

JOHN J. WILLIAMSON, OF BOSTON, MASSACHUSETTS.

## METHOD OF MAKING ELECTRICAL CONDUCTORS.

SPECIFICATION forming part of Letters Patent No. 319,536, dated June 9, 1885.

Application filed July 9, 1884. (No model.)

*To all whom it may concern:*

Be it known that I, JOHN J. WILLIAMSON, of Boston, in the county of Suffolk and State of Massachusetts, a citizen of the United States, 5 have invented a certain new and useful Improvement in Electrical Conductors and in the Manufacture Thereof, of which the following is a specification..

An electrical conductor, being in most instances suspended on poles above the ground, should be of a high tensile strength and high modulus of elasticity, to enable it to suspend its own weight between the supporting-poles and resist the stretching effect of wind and 15 gravity, and it should also be of high conductive properties, and as little as possible liable to disturbance by induction from adjacent electrical conductors. Inasmuch as the metals which are best for electrical conductors are of 20 low tensile strength and very low modulus of elasticity, and the metals which are of high tensile strength and high modulus of elasticity are of inferior electrical conductivity, it is evident that a combination of metals, 25 one for strength and one for conductivity, is desirable, if it should be practical. This fact has long been recognized.

In order to make a combination of two metals, one of high conductivity and the other of 30 high tensile strength, which shall be the best for all practical purposes, it is desirable that the coefficients of expansion between the two constituents of the conductor should be as nearly alike as possible, and also that the 35 metals should not be so different in their natures as to originate a local galvanic action under the influence of atmospheric moisture and atmospheric chemical impurities which would corrode the electro-negative metal and 40 injure its tensile strength. The only commercially practical metal of highest conductivity for the ordinary purposes of an electrical conductor is copper, whose modulus of conductivity is only exceeded by silver, while 45 its price is comparatively low, even as measured with iron. The coefficient of expansion of copper is but slightly influenced by alloying it, while its tensile strength is vastly increased, and its conductivity is vastly decreased by alloying. A copper-cored or copper-covered wire is therefore indicated by the 50 conditions required, and the core or cover of

metal of high tensile strength and low conductivity is indicated to be made of an alloy of copper which shall retain the copper coefficient of expansion and be superior in all properties except that of conductivity. All, or nearly all, the alloys of copper with other metals have their temperatures of fusion less than that of copper. All, or nearly all, of 55 the alloys of copper with other metals have physical properties equal or superior to copper for hot working. The alloys of useful strength which I propose to use are what are known as aluminum, bismuth, carbon and ferro-zinc bronzes, the Muntz metal, the Delta metal, which is a ferro-zinc bronze or brass, the Ajax metal, which is a composition 60 indifferently classified as bronze or brass, manganese and phosphor bronzes, sterro-metal, 65 nickel and silicon bronzes, because these have or can be made of high tensile strength and high modulus of elasticity, and are very little subject to corrosion, and are but slightly electro-negative to copper; but it will be obvious 70 that any strong alloy of copper which is of about the same coefficient of expansion as copper will be the equivalent of these. While such conductors will be more expensive than the compound conductors of iron or steel and 75 copper in the first instance, they will probably in the long run not be much more expensive, because more durable.

In making the electrical conductor with a copper interior and an exterior made of 80 those bronzes, brasses, or alloys, they may be so put together as to have copper and bronze in contact, but not united. There will be but slight difference in tensile strength or conductivity in these two cases; but it is probable that 85 the conductor of united metals would be better in some respects than a conductor of dissociated metals. The difference in manipulation to produce dissociation would practically be the difference between putting the two metals 90 together, both of them being heated to about the fusing temperature of the most fusible metal for association or putting them together, with a considerable difference between these 95 temperatures for dissociation.

The process of making these compound electrical conductors has several stages: first, the formation of the ingot; second, its reduction into billets, bars, and rods; and, third, the re- 100

duction of the rods into wire. The formation of the ingot is of the most consequence; but there is a special manipulation required whenever a partially-reduced ingot is cut for convenience of manipulation in further stages.

By reference to the drawings, Figure 1 shows a mold, C, for casting the most fusible metal around the copper bolt E set up within it. This copper bolt E is to form the conducting thread of the finished wire. It is set up in the center of the mold along its axis a short distance from the bottom, and should be supported upon a small block or standard of metal, F, similar to that which is about to be poured, 15 or it may be upon wires of such metal so as to hold its proper position within the mold, and allow the fluid metal to flow all around it. I prefer to support it on a small pedestal of the metal about to be poured. This bolt of copper, E, must be set a little shorter than the ingot-mold, so that the molten metal, D, may flow over its top and inclose the upper end of the copper as well as under the bottom of the copper bolt, inclosing that. The atmospheric action 20 which takes place during the working of an ingot thus made will be simply the surface action upon the incasing metal, and will not affect the copper interior at all, while the work to which the ingot is subjected will be work 25 that affects the mass throughout and fibrizes the copper and improves its conductive qualities, besides which, when the copper is completely inclosed, inequality in the reduction of the copper or of the alloyed exterior will be 30 avoided or reduced to a minimum, while if it were unconfined at one or both ends there would be a liability to unequal reduction, and when the copper bolt is put in hot for the purpose of having the two metals united in the 35 finished article this covering or boxing in of the copper will be particularly important. When the copper bolt is put in hot, of course the exterior casing should be poured as rapidly as possible.

45 In case it is desired to make the bronze exterior of the ingot first, and then pour molten copper into it, this may be done; but in such case the shell would require to be chilled on its exterior while the copper was poured and 50 for some little time after, so that the copper should not fuse the more fusible metal into which it is cast, but its excessive heat should be rapidly conducted off; and this chill should be applied as well to the bottom of the hollow 55 ingot as to the sides, because of the danger of molten copper eating out the bottom of the ingot; but a small section of properly-prepared asbestos or other very inferior conductor could be placed upon the bottom of the cavity in the 60 ingot, and this limited quantity of impurity would be cut off subsequently in the clipping of the billets, bars, or rods; and in case molten copper was inserted into the cavity of the more fusible ingot, as above described, the upper 65 end of the ingot should be subsequently closed by molten metal of the character of the exte-

rior by plugging with refractory material or by closing over the end in any proper way.

If desired to produce an electrical conductor with a copper section and a center of stronger metal, a copper ingot should be first cast hollow, as shown in Fig. 2, A, and its center filled with the more fusible metal, B; and if desired to have a union between the two different metals the hollow copper ingot should be heated 70 to a proper temperature. So, also, copper may be poured upon a solid bar of the alloy or bronze, and if done quickly, and there is not too much copper, the alloy will probably not be taken up by the copper; but I do not recommend this as the best way of doing. The finished wire is shown at Fig. 3, in which A is the exterior metal, and B the interior, both of the same general nature, but differing only in electric conductivity. In case the copper absorbs the alloy, or is absorbed by it, both the electric conditions will be injured and the tensile strength will be impaired, so that it is desirable that the two metals should be kept from anything more than mere surface union, 85 substantially likesweating together. Of course the surface of that part of the ingot which is first prepared, whether it be the coring part or whether it be the exterior, should be clean of sand, scale, or other impurities, and should 90 be in such a condition as not to have much air adherent to it. If these surfaces are thoroughly cleaned from scale and then washed with oil and lamp-black, or other substances well known to copper-workers for making such a 100 coating, these substances will be taken off by the molten metal and floated upon it or destroyed, removing all the air from the surfaces at the same time, and thus the surface of the original part of the ingot, whether 105 it be the bolt for the center of the hollow ingot for the exterior, will be practically chemically clean for its contact with the part subsequently to be poured into it or around it. This ingot, so made, has closed ends, and may 110 be worked under the hammer or in rolls, as if it were entirely composed of the metal which forms its exterior; if that be the most fusible metal, or, at any rate, at the working temperature of the most fusible metal, or, if copper, 115 on the exterior metal, and its working temperature be the lower at the copper-working temperature, the ingot having the metal of highest tensile strength, least conductivity, and least fusing temperature on the exterior, will 120 be the preferable ingot to work, as copper is not a good metal to work at high heats. This ingot is then reduced to billets, bars, and rods in the usual way of such reduction; but in case 125 it is necessary to cut any of these products because they are too long, care must be taken before reheating or making use of either of the pieces with a cut end to hammer up the end, so as to close the exterior metal over the interior metal as much as possible, and thereby 130 eliminate the exposure of the inclosed metal to the atmosphere and keep it in the same con-

dition and relative position in which it was. Wire is then drawn from the rods formed in the usual way, and this wire, if it be made from the ingot with the bronze exterior and the copper interior, will have a comparatively-uniform filament of copper throughout its entire length, surrounded by a casing of bronze of much greater tensile strength, preserving the copper from atmospheric action, and also insulating it to a certain degree, and so protecting it from induction and what might be called the "vagabond currents," which leak from adjacent wires and disturb the usefulness of an electric conductor.

15 I have claimed in an application filed January 23, 1884, and allowed June 17, 1884, the method of producing electric conducting-wires composed of copper and copper alloys by casting or pouring molten fluid copper or copper alloys on and around a solid bar or within a hollow ingot of copper or copper alloy, said solid bar or hollow ingot being, while the casting is effected, at such high degree of temperature that the pouring of molten metal on

20

it will produce metallic fusion between the 25 sections, and afterward reducing such ingot to the diameter proper for electrical conductors. I do not wish to be understood as herein claiming the same.

Having thus fully described my invention, 30 I claim and desire to secure by Letters Patent of the United States—

The method of producing electric conducting-wires composed of copper and copper alloys by casting or pouring molten fluid copper 35 or copper alloys to and around a solid bar or within a hollow ingot of copper or copper alloy, said solid bar or hollow ingot being, while the casting is effected, at such degree of temperature that no metallic fusion between the 40 sections is produced, and afterward reducing such ingot to the diameter proper for electrical conductors by the usual suitable means.

JOHN J. WILLIAMSON.

Witnesses:

F. F. RAYMOND, 2d  
FRED. B. DOLAN.